

March 12, 1968

L. KUNSAGI ET AL

3,372,565

## CORRUGATION FORMING BY EXPLOSIVES

Filed April 13, 1965

4 Sheets-Sheet 1



INVENTORS  
LASZLO KUNSAGI  
WILLIAM R. APBLETT  
IRWIN BERMAN  
JOSEPH H. HEIFETZ  
BYRAM J. MAJOL  
BY Richard H. Thomas  
ATTORNEY

March 12, 1968

L. KUNSGI ET AL

3,372,565

CORRUGATION FORMING BY EXPLOSIVES

Filed April 13, 1965

4 Sheets-Sheet 2

Fig. 5.



Fig. 6.



Fig. 7.

INVENTORS  
LASZLO KUNSGI  
WILLIAM R. APBLETT  
IRWIN BERMAN  
JOSEPH H. HEIFETZ  
BY RAM J. MAJOL  
BY Richard H. Thomas  
ATTORNEY

March 12, 1968

L. KUNSAGI ET AL

3,372,565

CORRUGATION FORMING BY EXPLOSIVES

Filed April 13, 1965

4 Sheets-Sheet 3

Fig. 8.



Fig. 9.

INVENTORS  
LASZLO KUNSAGI  
WILLIAM R. APBLETT  
IRWIN BERMAN  
JOSEPH H. HEIFETZ  
BYRAM J. MAJOL

BY

*Richard H. Thomas*  
ATTORNEY

March 12, 1968

L. KUNSGI ETAL

3,372,565

CORRUGATION FORMING BY EXPLOSIVES

Filed April 13, 1965

4 Sheets-Sheet 4

Fig.10.



Fig. 11.



Fig. 12.



Fig. 13.

INVENTORS  
LASZLO KUNSGI  
WILLIAM R. APBLETT  
IRWIN BERMAN  
JOSEPH H. HEIFETZ  
BYRAM J. MAJOL

*Richard H. Thomas*  
ATTORNEY

1

3,372,565

**CORRUGATION FORMING BY EXPLOSIVES**  
Laszlo Kunsagi, New York, N.Y., William R. Applett,  
Metuchen, N.J., Irwin Berman, Bronx, N.Y., and  
Joseph H. Heifetz, Fort Lee, and Byram J. Magol, Con-  
vent, N.J., assignors to Foster Wheeler Corporation,  
New York, N.Y., a corporation of New York  
Filed Apr. 13, 1965, Ser. No. 447,709  
15 Claims. (Cl. 72—56)

## ABSTRACT OF THE DISCLOSURE

A method and apparatus for corrugating panels by the use of explosive wherein the explosive is limited in amount so that grooves in the panel are substantially free-formed.

This invention relates to the fabrication of high strength panels. In particular, it relates to a method involving free forming of high strength corrugated panels by explosive.

Corrugated paneling is advantageous from considerations of strength and design. In the past, heavy dies have been used to fabricate contoured panels in conjunction with both press formation, and with explosive formation. Where the panels to be formed are limited in number, the expense and inconvenience of die fabrication may be prohibitive. Even with the manufacture of a large number of panels, the cost of heavy dies may be a burden. Also, where the contour design configuration is changed from panel to panel or where the panel sizes vary, die formation is highly undesirable. A further disadvantage is inherent in press formation methods utilized in conjunction with conventional dies, since panel shrinkage may occur making it impossible to pre-size the panel for installation prior to contour forming.

Therefore, it is an object of the present invention to provide economical and convenient methods for the manufacture of corrugated panels.

It is also an object of the present invention to provide a method in which the use of conventional contour or forming dies is avoided.

It is a further object of the present invention to provide a method for the production of ultra-high strength contoured panels which are flexible in the plane of the panel.

It is another object of the invention to provide a method by which panels can be pre-sized and subsequently formed, without altering the over-all panel size during forming.

In accordance with the present invention, shaped charges are supported against or closely adjacent to a panel to be formed, with major portions of the explosive along the lines of the contours to be produced, the shape and sizes of the charges being dictated by preselected shapes of the contours. The charges are simultaneously detonated in a suitable medium to develop localized shock waves which are transmitted to the adjacent area on the panel. The latter is supported at points remote from the contour forming explosive, so that the shock waves produce a rapid and localized substantially free-forming expansion of the panel in the adjacent areas, developing high strength corrugations. By virtue of localization of the expansion, the overall dimensions of the panel are not changed.

Employing this method, various shaped contoured panels, including high strength corrugated panels, are conveniently and economically manufactured. A limited number of contoured panels may be simply formed by placing the explosive adjacent the areas where the contours are desired. The contoured panels may also be formed after the panels are initially sized for assembly since the over-all dimensions do not change during the forming.

2

The invention and these and other advantages will appear more fully from the following description and accompanying drawings, wherein:

FIGURE 1 is a plan view of an apparatus for producing a corrugated panel by explosive forming of shaped charges in accordance with the invention;

FIGURE 2 is a section view taken along line 2—2 of FIG. 1;

FIGURE 2A is an enlarged section view taken on line 2A—2A of FIG. 1;

FIGURE 3 is a section view taken along line 3—3 of FIG. 1;

FIGURE 4 is an enlarged section view illustrating details of the apparatus of FIG. 1 and the method in accordance with the invention;

FIGURE 5 is a section view corresponding to FIG. 2 illustrating an embodiment in accordance with the invention;

FIGURE 6 is an enlarged section view of a portion of the apparatus of FIG. 5 illustrating details of the embodiment and steps of the method in accordance with the invention;

FIGURE 7 shows formed panel corrugations and contains a graph providing evidence of operativeness of the method and apparatus of the invention; and,

FIGURES 8—13 illustrate applications for corrugated panels produced in accordance with the invention.

Referring to the drawings and more particularly to FIGS. 1—4 there is shown the basic method and apparatus for producing high strength corrugated panels by substantially free-forming of the panels with shaped explosive charges. Any suitable explosive, such as the strips generally designated 12, are placed on a pre-sized panel 14 of any ductile material, such as type 301 austenitic stainless steel, in a predetermined layout. They are placed in parallel in FIG. 1 directly against the panel 14 to produce the parallel corrugations shown in FIGS. 7 and 8. Explosive is available at 20, 30, 40, 50, 60 and 100 grains per foot, and the concentration used depends on the thickness and material of the panel, depth and closeness of corrugations desired, and other factors which will become apparent. As an alternative, the explosive may be cast in sheet form with major concentrations of explosive defining a predetermined layout to produce the corrugations of FIGS. 7 and 8. In this respect, it should be noted that the layout of explosive, whether in strip form or cast sheet form, may be designed to produce parallel corrugations or corrugations of any other predetermined pattern.

In this example, the concentration used was twenty-five grains per foot. The panel was 16 gage austenitic stainless steel having a width of about forty inches, a length of about forty-two inches, and an average thickness of .050 inch, and was formed with the substantially uniform sinusoidal corrugations shown in FIG. 7, about  $\frac{1}{2}$  inch in depth on four inch centers, leaving about ten inches of flat plate area (not shown) on each side of the panel. FIG. 7 shows the variation in thickness in the panel following forming, averaging less than .002 inch with a maximum variation of .004 inch. Changes in width and length dimensions were negligible.

Referring again to FIGS. 1—4, a reinforced concrete base 16 is constructed having a plate 18 secured to the upper surface thereof and made substantially horizontal. Experience has shown that it is desirable to maintain the level of the plate within a tolerance of  $\pm \frac{1}{16}$  inch. Half rounds 20 are suitably supported on the plate 18 spaced from the upper surface of the plate and from each other. In this example, the half rounds are on 4 inch centers, are parallel to each other and have a diameter in the order of two inches. Their spacing from the surface of the plate is sufficient such that contact of the panel 14 downwardly

with the plate under the force of explosive is avoided; i.e., expansion of the panel is substantially free-forming.

The panel 14 to be formed is placed on top of the half rounds, and intermediate the half rounds, also on four inch centers, the explosive strips 12 are located on top of the panel. A thin gage polyethylene sheet 22 is then laid over the panel and explosive and is backed up by loose end bars 24 forming a continuous dam adjacent the periphery of the panel 14. A suitable force transmitting fluid 26, for instance water, fills the inside of the dam covering the explosive strips 12.

At opposite ends of the spaces 28 between half rounds 20, T's 30 fill the span between the half rounds and abut the underside of the panel 14, extending between the panel and the surface of plate 18. As shown in FIG. 3, the T's are provided with rounded leading edges 32 facing inwardly towards spaces 28, their purpose being to assist in the formation of the corrugations and to avoid the formation of sharp edges.

The ends of charges 12 may be extended over the flat surfaces of the T's for the purpose of holding down the panel on detonation. Additional hold-down charges 36 should be used over the outermost or end half rounds 38 for the same purpose, and if desired, intermediate charges 34 (FIG. 2A) may be used over the intermediate half rounds for this purpose. As mentioned above, the panel is dimensioned so that the end half rounds 38 preferably are at least ten inches inside of the ends of the panel. Experience has shown that this dimension is instrumental in avoiding panel shrinkage. By the same token, providing a distance between the ends of the corrugations and the panel side edges of about ten inches avoids distortion and side to side shrinkage.

At this point it should be noted that only a relatively small overall amount of hold-down explosive is used as compared to the overall amount of explosive used in forming strips 12, to prevent pull-in along the edges of the panel and consequent panel shrinkage. In this example, a charge concentration of twenty grains per foot sufficed. Generally, the intermediate hold-down charges will be in the order of twenty grains per foot.

On the method of FIGS. 1-4, it should be noted that the panels were first dimensioned and laid out for length, number and location of corrugations, and the explosive strips 12 were dimensioned, sized and located according to layout, in parallel alignment, although other patterns are within the scope of this application. The parallel alignment is necessary to obtain a sinusoidal configuration. In placing the panel on the half rounds, the explosive strips 12 should coincide with the center lines of the short T's 30, with preferably an overlap of the strips on to the T's, for the purpose of providing additional hold-down. Where a shallower corrugation is desired, about one inch of clear space may be provided between the ends of the explosive and the T inboard ends 32.

Following set-up of the assembly, the explosive forming and hold-down strips are simultaneously detonated by suitable equipment 40 (FIG. 3), the detonation traveling at the same rate down the length of each charge progressing from common charge ends 42. Pressure waves are transmitted through the liquid transmitting medium 26 to the panel 14 along parallel paths corresponding to the charge positions. The impacting waves simultaneously produce uniform corrugated depressions 44, shown in dotted lines in FIGS. 2 and 4, which are substantially free-formed except at the inboard ends of T's 30.

As a result of the linear shape of the charges and the proximity of the charges to the panel, the impacting pressure waves are localized relative to the panel expanding only those portions of the panel directly adjacent the charges. Also, due to the narrow width of the charges relative to the overall panel dimensions and the localized and rapid strain rate expansion, the overall dimensions of the formed sheets after detonation remain the same as

they were prior to detonation. No clamps are required to inhibit overall dimensional changes in any respect.

FIG. 4 shows further details in the construction of the half rounds and supports therefor. Elongated support blocks 46 are welded or suitably held on plate 18 and the half rounds 20 are bolted to the blocks.

Other modes of construction are suitable in accordance with the invention to allow for a substantially free-formed corrugation, for instance the apparatus of FIGS. 5 and 6. In this embodiment, a reinforced concrete foundation 50 is constructed having a plurality of parallel closely adjacent V grooves 52, on four inch centers, provided with steel plate cladding 54 to align pipes 56. The level of the foundation is again maintained within a tolerance of  $\pm \frac{1}{16}$ ".

Two inch diameter pipes 56 are placed in the V grooves and short T's 58 are placed upright in the spaces 60 between the pipes in positions corresponding to the terminus or end of each corrugation. The inboard ends of the short T's are suitably rounded to prevent the T's from cutting into the panel during forming. On the left and right ends of the panel 62, the first and last T's 64 and 66 extend substantially the full length of the foundation. In effect, these long T's will be about four inches or one corrugation width from the first and last corrugations made in the panel. The upper surfaces of the T's and pipes coincide in altitude.

The panel 62 to be formed is placed over the pipes and T's resting against both, and is located so that all lengths of explosive 68 coincide with the center lines of the spaces between the pipes (or center lines between opposed short T's). Again, the short T's preferably are located so that there is a slight overlap between the ends of the explosive and inboard ends of the T's. The end lengths 70 and 72 of explosive are placed directly over the center lines of the long T's, 64 and 66. An overow water dam 74 is placed over the work sheet, made up of a supporting frame as shown and the area within the dam is filled with water 76 to overflowing so that the level of water is about two inches.

Occasionally, a primacord charge will fail to detonate. Mistakes due to misfires can readily be corrected without damage to adjacent corrugations by using wet sand as a transmitting medium. As an example, referring to FIG. 6, where the pipes 56 are on four inch centers, two small primacord strips 78 and 80 (20-25 grains per foot) are placed in parallel approximately a half inch apart along the center line between the pipes 56. A layer of moist sand 82 is placed over the strips, and the strips are detonated in the usual manner. Following detonation, it is difficult by visual inspection to note the correction, and any difference in successive corrugations. In this respect, moist sand is preferred in that the charge force is slightly more localized.

FIG. 8 illustrates a roof panel for a large pressurized land boiler made from an 18 gage carbon steel sheet by the method of the invention. The corrugations again are on four inch centers, and provide a sinusoidal configuration. An average flat area ten inches wide along each side of the panel was sufficient to avoid side and length dimensional changes in the panel during forming, although in this instance, the sides were sheared to provide the finished dimensions. The amount of flat area on each side of the panel is critical to avoid dimensional changes, but varies slightly depending upon thickness of the panel and depth, width and length of corrugations.

The corrugations make an angle of 10° with the sides of the panel, illustrating that any angle corrugation can be made. In this instance, the angle was selected for drainage reasons. It was found that the corrugations provide substantially greater strength against bending than does a conventional non-corrugated 11 gage flat plate. An essentially flat upper surface facilitates use of insulation with the panel, and the reduced over all weight

has the result that one man can install the panel, whereas, normal installation requires the presence of two men.

FIG. 9 shows seal plates made in accordance with the invention. These seal plates, also used in boilers, must resist high temperature service and corrosive conditions. The seal plates were made of 11 gage corten steel and were corrugated to depths of  $\frac{5}{8}$  inch to  $\frac{3}{4}$  inch overall using the method of the invention. Explosive, having 60 grains per foot in a water depth of 3 inches, provided the desired force. The seal plates were subsequently oven tempered to reinstate their corrosion resisting properties, and were edge cut so that the corrugations run through to one edge while three edges remain flat. This provided a solution to the problem of cracking of the seal plates due to large temperature differences between the fixed and free edges.

The application of FIG. 10 concerns drip lips used in high temperature and highly corrosive boiler installations, designed to provide a run-off for fluid flowing into a deaerator feedwater storage vessel. The drip lips are 20 made of 304 annealed 11 gage stainless steel, and in conventional applications consist of flat panels bolted along an upper edge to a suitable rigid support. Under high temperature service, the drip lips presently used have a life expectancy of a few years due to a differential 25 expansion between the main portion of the lips relative to the bolted edge.

By the invention, the drip lips are provided with corrugations in the main portion thereof and along the edge removed from the bolted edge, which permits differential 30 expansion. Using conventional methods for making corrugations, it would be necessary to make the corrugations the full length or width (depending on the direction in which they extend) of the panels. By the invention, corrugations running along only the middle of the panel are made, and then the panel is cut in half, as shown. In this way, a drip lip is provided having a flat edge area for bolting to the support with the rest of the sheet and lower edge corrugated.

FIGS. 11-13 show a partition plate construction for feedwater heaters, of the type described in application Ser. No. 331,739, filed Dec. 19, 1963 by Edward Vogt. The plates are formed of 3 sections, welded together, two end sections (FIG. 11) and a middle section (FIG. 12). The added strength afforded by the corrugations permits the use of a thinner gage material than that conventionally used. This in turn reduces stress concentrations along lines of connection between the partition plate and heater shell, the latter being of high strength relatively thick steel.

Tests have shown that uniform repeatable corrugations can be formed on ductile materials such as mild steel, low carbon steel and corten steel, and stainless steel in thicknesses ranging from 18 gage (.049 inch) to 10 gage (0.1345 inch) with indications that the spacing of corrugations can be varied and the thickness of the material increased without difficulty. The shape of the panel to be corrugated and non-uniformity in length requirements present no problem.

The following table is illustrative of corrugated panels made in accordance with the invention.

Although the invention has been described with a certain degree of particularity, it is understood that numerous changes in the details of construction and the combination and arrangements of parts may be resorted to without departing from the spirit and the scope of the invention as hereinafter claimed.

What is claimed is:

1. A method for strengthening a metallic panel by explosively forming a plurality of elongated grooves in the panel, said forming being without the use of dies having the configuration of the panel so formed; comprising the steps of

positioning the panel over a supporting structure, said structure including a plurality of elongated raised spaced apart supports having rounded upper surfaces, the surfaces extending at least the lengths of the grooves desired and the upper surfaces thereof being elevated above the rest of the supporting structure a distance greater than the depths of said grooves; disposing explosive on the panel with at least a greater amount of explosive intermediate said supports and extending at least the lengths of the grooves; detonating the explosive to form the grooves; the amount of explosive intermediate the supports being less than that which would cause the panel to come into substantial contact with said supporting structure other than with the upper surfaces of said spaced apart supports whereby the forming of the grooves is substantially free and unrestricted by said supporting structure.

2. A method according to claim 1 wherein the detonating explosive is in the form of elongated narrow strips of explosive in juxtaposition with the panel and disposed along a plane centered between the supports, the width 35 of the explosive being narrow relative the overall dimensions of the panel to confine the explosive force substantially to the plane centered between the supports,

further including additional elongated narrow strips of explosive of narrow width relative the overall dimensions of the panel in juxtaposition with the panel and along parallel planes centered over said supports, functioning to hold-down the panel, the method further including the step of detonating said additional strips of explosive simultaneous with the detonation of the first-mentioned strips of explosive.

3. A method according to claim 1 wherein said elongated supports are in parallel alignment and on at least four inch centers;

the explosive intermediate said supports having a concentration of at least 20 grains per foot sufficient to form substantially sinusoidal corrugations in said panel.

4. A method according to claim 1 wherein said explosive is detonated within a shock wave transmitting 55 medium.

5. A method according to claim 1 including the step of supporting the panel between the spaced apart supports at the ends of the grooves to be formed to limit the lengths of the grooves.

6. A method for corrugating metallic flat panels having opposed ends comprising the steps of

| Use Intended                                      | Plate Thickness    | Material                | Explosive<br>Grains per<br>Foot | Water<br>Depth (in.) | Depth of<br>Corrugation<br>(in.) | Spacing of<br>Corrugation<br>$\frac{C}{C}$ to $\frac{C}{C}$ (in.) |
|---------------------------------------------------|--------------------|-------------------------|---------------------------------|----------------------|----------------------------------|-------------------------------------------------------------------|
| Test                                              | 11 Gage (.120 in.) | Corten                  | 60                              | >1.5                 | $\frac{5}{8}$                    | 4                                                                 |
| Do                                                | do                 | Low Carbon Steel        | 60                              | >2                   | $\frac{5}{8}$                    | 4                                                                 |
| Boiler Roof Panels                                | do                 | Carbon Steel            | 50                              | 2 $\frac{1}{2}$      | $\frac{5}{8}$                    | 4                                                                 |
| Boiler                                            | 18 Gage (.049 in.) | do                      | 25                              | $\frac{5}{8}$        | $\frac{5}{8}$                    | 4                                                                 |
| Boiler Drip Lips                                  | 11 Gage (.120 in.) | No. 304 Stainless Steel | 100                             | 3                    | $\frac{5}{8}$ -1                 | 4                                                                 |
| Boiler Seal Plates                                | do                 | Corten Steel            | 60                              | 3                    | $\frac{5}{8}$ - $\frac{3}{4}$    | 4                                                                 |
| Pass Partition Plates for Condensers <sup>1</sup> | 10 Gage            | Low Carbon              | 60                              | 3                    | $\frac{5}{8}$                    | 4                                                                 |
| Pressurized Boiler Panel <sup>2</sup>             | 16 Gage (.065 in.) | No. 321 Stainless Steel | 60                              | 2                    | 1                                | 4                                                                 |

<sup>1</sup> Resists 20 p.s.i. differential better than present  $\frac{1}{2}$  in. flat plate.

<sup>2</sup> Resists 160 inches water pressures without excessive bowing.

horizontally leveling the panels on a supporting structure including a plurality of elongated parallel spaced apart supports having rounded upper surfaces, the supports extending at least the lengths of the corrugations desired and being in side-by-side relationship between the panel ends, the upper surfaces of said supports further being elevated above the rest of the supporting structure a distance greater than the depths of the panel corrugations;

disposing a first series of continuous concentrations of explosive on the panel intermediate said supports having a charge concentration of at least 20 grains per foot, the concentrations of explosive being at least coextensive with the lengths of corrugations desired; providing additional supports spaced from said parallel supports and from the panel ends but between the spaced supports and panel ends;

disposing a second series of continuous concentrations of hold-down explosive over said additional supports; simultaneously detonating the first and second series of explosive;

the improvement comprising detonating only limited amounts of explosive so that forming of the grooves is substantially free and unrestricted by the supporting structure.

7. A method of explosively forming a narrow contour in a ductile panel, comprising the steps of disposing an elongated continuous strip of explosive charge in juxtaposition with the panel, the width of the strip being small relative the over-all dimensions of the panel,

supporting the panel over a supporting structure including a plurality of raised spaced apart supports so that the portions of the panel adjacent the explosive strip are in spaced relation with the supports, the upper surfaces of the supports being elevated above the rest of the supporting structure a distance greater than the depth of said contour,

detonating the explosive strip from one end of the strip to cause the explosive to travel down the length of the strip thereby progressively forming a contour in the panel along the portions of the panel adjacent the strip, wherein only a limited amount of explosive is detonated so that forming of the contours is substantially free and unrestricted by the supporting structure.

8. A method according to claim 7 further comprising the steps of constructing a temporary retaining ridge around the portion of the panel where the contour is to be formed, filling the portion bounded by the ridge with a liquid transmitting medium so that the continuous strip is at least partially immersed in the liquid.

9. A method of explosively forming narrow parallel contours in a ductile panel, comprising the steps of disposing a first series of elongated continuous parallel strips of explosive charges in juxtaposition with the panel, the width of the strips being small relative the overall dimensions of the panel,

supporting the panel over a supporting structure including a plurality of raised spaced apart supports so that the portions of the panel adjacent the explosive strips are in spaced relation with the supports, the upper surfaces of the supports being elevated above the rest of the supporting structure a distance greater than the depths of said contours,

simultaneously detonating the explosive strips and initiating detonation of each strip at a point of intersection between the strip and a line which is perpendicular to all the strips to cause the explosions to travel uniformly down the strips thereby progressively forming parallel contours in the panel along portions of the panel adjacent the strips, wherein only a limited amount of explosive is detonated so that forming of

10

15

20

25

30

35

40

45

50

55

60

65

70

75

the contours is substantially free and unrestricted by the supporting structure.

10. A method of explosively forming parallel contours to form a sinusoidal configuration in a ductile panel, comprising the steps of

disposing elongated continuous parallel strips of explosive charges in juxtaposition with the panel, the width of the strips being small relative the over-all dimensions of the panel, the strips further being equal distances apart and having an equal number of grains of explosive per foot of strip;

supporting the panel over a supporting structure including a plurality of raised spaced apart supports so that the portions of the panel adjacent the explosive strips are in spaced relation with the supports, the supports being intermediate the strips, the upper surfaces of the supports further being elevated above the rest of the supporting structure a distance greater than the depths of said contours;

simultaneously detonating the explosive strips and initiating detonation of each strip at a point of intersection between the strip and a line which is perpendicular to all the strips to cause the explosions to travel down the strips thereby progressively forming sinusoidal parallel contours in the panel along portions of the panel adjacent the strips wherein only a limited amount of explosive is detonated so that forming of the contours is substantially free and unrestricted by the supporting structure.

11. Apparatus for explosively forming metallic panels comprising

a substantially horizontal base;

a plurality of elongated spaced apart supports each having a rounded upper surface, the support upper surfaces spaced from said base and defining a substantially horizontal plane;

additional support means in said plane spanning the spaces between the spaced apart supports at the ends of predetermined distances corresponding to the lengths of grooves desired in the panel, the additional support means having rounded inwardly facing edges;

the plane of the support upper surfaces being spaced a distance from the base sufficient such that grooves in the panel intermediate the supports are substantially free formed.

12. Apparatus according to claim 11 wherein said spaced apart supports are parallel and on at least four inch centers.

13. A method for forming corrugated steel panels having a panel thickness less than 0.25 inch, the corrugations being less than one and one half inches deep, comprising the steps of

horizontally positioning a flat panel so that it rests against a plurality of elongated parallel spaced apart supports having rounded upper surfaces with approximately a one inch radius, the supports extending the lengths of the corrugations desired and being raised sufficiently so that the corrugations are substantially free formed;

disposing a first series of continuous concentrations of explosive on the panel having a charge concentration of at least 20 grains per foot, the charge concentrations being at least coextensive with the lengths of corrugations desired and intermediate said supports;

disposing a second series of continuous concentrations of explosive on the panel having charge concentrations of at least 20 grains per foot, the second series of concentrations being over lines of contact of said supports and panel, at least two of said second series of concentrations being between the panel ends and the endmost corrugations;

simultaneously detonating the explosive concentrations from one end thereof to cause the explosions to travel

the lengths of the concentrations thereby progressively forming a plurality contour in the panel, the concentrations of explosive being separate from one another and narrow relative the distance from crest to crest of the panel contours.

14. A method according to claim 13 wherein said supports are in parallel relationship and on approximately four inch centers to produce corrugations having a substantially sinusoidal configuration.

15. A method according to claim 13 wherein the end-most corrugations are at least about ten inches from the panel ends.

## References Cited

## UNITED STATES PATENTS

|           |         |         |       |       |
|-----------|---------|---------|-------|-------|
| 2,935,038 | 5/1960  | Chatten | ----- | 72—56 |
| 3,060,879 | 10/1962 | Staba   | ----- | 72—56 |
| 3,120,827 | 2/1964  | Abegg   | ----- | 72—60 |
| 3,238,753 | 3/1966  | Benatar | ----- | 72—56 |

RICHARD J. HERBST, *Primary Examiner.*

10 K. C. DECKER, *Assistant Examiner.*